

## UNITED STATES PATENT OFFICE.

FOSTER MILLIKEN, OF LAWRENCE, NEW YORK.

## ALLOY.

No Drawing.

Application filed October 8, 1919. Serial No. 329,165.

To all whom it may concern:

Be it known that I, FOSTER MILLIKEN, a citizen of the United States, and a resident of Lawrence, in the county of Nassau and 5 State of New York, have invented a new and Improved Alloy, of which the following is a full, clear, and exact description.

The object of the invention is to provide a new and improved alloy capable of being 10 rolled, drawn, forged or worked in other ways while being cold to form rods, wires, tubing and the like.

The alloy contains the following metals in substantially the following proportions, 15 namely:

|                     |                 |
|---------------------|-----------------|
| Copper              | 60-70 per cent. |
| Nickel              | 9-12 per cent.  |
| Zinc                | 19-24 per cent. |
| Iron                | 1-2½ per cent.  |
| Trace of manganese. |                 |

These metals are melted together and the resultant alloy is adapted for cold working and has the additional advantage of being 25 acid resisting. It is understood that the iron used is not alloyed with any other element before combining it with the other ingredients.

The addition of the manganese toughens 30 the alloy and not only changes the physical characteristics, that is, its tensile strength, its elastic limit, its elongation and reduc-

tion of area, but has a decided effect on the chemical resisting qualities of the alloy.

Tests of the new alloy have produced the 35 following results:

## Rods.

|                   | Unannealed. | Annealed. | 40 |
|-------------------|-------------|-----------|----|
| Tensile strength  | 121.200     | 91.200    |    |
| Elastic limit     | 112.600     | 63.800    |    |
| Elongation        | 8.6%        | 32.6%     |    |
| Reduction in area | 10.2%       | 54.5%     |    |

## Wire.

|                   |         |
|-------------------|---------|
| Tensile strength  | 162.800 |
| Reduction in area | 48.2%   |

This alloy differs from the one described in the Letters Patent of the United States, 50 No. 1,814,417, granted to me on August 26, 1919, in that it has a high percentage of copper, a lower percentage of zinc, and but a trace of manganese.

Having thus described my invention, I 55 claim as new and desire to secure by Letters Patent:

An alloy consisting of the following ingredients in substantially the following proportions: copper 60 to 70 per cent, nickel 9 60 to 12 per cent, zinc 19 to 24 per cent, iron 1 to 2½ per cent, and a trace of manganese.

FOSTER MILLIKEN.